# EUROPEAN PATENT SPECIFICATION

(11) **EP 0 943 029 B1**
(45) Date of publication and mention of the grant of the patent: **31.07.2002**
(21) Application number: 97949841.7
(22) Date of filing: 03.12.1997
(51) Int. Cl.: D06N 3/00, D06N 3/04, D06N 7/00, B05D 3/06

(54) **REINFORCEMENT MATERIALS AND METHODS FOR THE PREPARATION THEREOF**
VERSTÄRKUNGSMATERIALIEN UND VERFAHREN ZU IHRER HERSTELLUNG
MATERIAUX DE RENFORCEMENT ET LEURS PROCEDES DE PREPARATION

(30) Priority: 04.12.1996 NL 1004692
(43) Date of publication of application: 22.09.1999
(73) Proprietor: N.V. Syncoglas S.A., 9240 Zele (BE)
(72) Inventor: GODDERIS, Eric, B-9041 Gent (BE)
(74) Representative: Van Someren, Petronella F. H. M.
(86) International application number: BE9700131
(87) International publication number: WO9824966

(56) References cited:
- DATABASE WPI Section Ch, Week 9519 Derwent Publications Ltd., London, GB; Class A32, AN 95-144199 XP002037268 & JP 07 068 542 A (SOMAR CORP) , 14 March 1995
- DATABASE WPI Section Ch, Week 9204 Derwent Publications Ltd., London, GB; Class A81, AN 92-029833 XP002037269 & JP 03 277 682 A (NICHIBAN KK) , 9 December 1991
- DATABASE WPI Section Ch, Week 9310 Derwent Publications Ltd., London, GB; Class A12, AN 93-080594 XP002037270 & JP 05 025 418 A (HITACHI CHEM CO LTD) , 2 February 1993
- DATABASE WPI Section Ch, Week 9437 Derwent Publications Ltd., London, GB; Class A81, AN 94-300025 XP002037271 & JP 06 228 512 A (OJI PAPER CO) , 16 August 1994

## Description

The present invention relates to a method for manufacturing a self-adhesive strengthening material and to the thus obtained material and its applications.

Cracks or deformations can occur in buildings and structural works such as roads, bridges, viaducts and the like owing to uneven expansion and shrinkage, settling of the building or structural work, too high a load and so on. A good example in road-building is the forming of ruts in asphalt roads due to overloading. Forming of cracks in buildings can for instance also occur in the finish thereof, such as in building materials applied therein such as gypsum plaster or cement plaster, or in floors, terraces, asphalt roofs, outside wall insulation systems and the like. In order to prevent this type of effect the building material used is generally strengthened by means of a strengthening material.

Known strengthening materials consist of open-mesh woven fabrics or webs, the fibres of which are generally protected against wear or the action of acids and/or bases by means of a resin. When used in building materials the strengthening material is then pressed into the preferably still wet base layer, whereafter a finishing layer is applied.

However, when the base layer is not or no longer wet, some form of fixing of the strengthening material to the base layer is still required. It is therefore known to apply a glue layer on one side after arranging and setting of the protective resin. This application of the glue layer generally takes place at the location of the works.

The drawback hereof, however, is that the applying of the glue layer requires an additional operation and extra material.

From JP-A-7,068,542 it is known to provide a reinforcing fibrous matrix impregnated with a sticky thermosetting resin. In order to make one side non-sticky, an additional layer of a thermoplastic resin is applied onto the sticky surface, thus requiring an additional step and material.

It is the object of the present invention to provide a new method for manufacturing a self-adhesive strengthening material, and also to provide a new strengthening material.

This is achieved by the invention with a method comprising the steps of:
a) providing a coarse-mesh net consisting at least partially of strengthening fibres;
b) at least partly encapsulating or impregnating the strengthening fibres of the net with a coating layer of an adhesive resin; and
c) making the resin non-adhering on one side of the net,
wherein the resin is sensitive to, or can be made sensitive to, UV-light, and making the resin non-adhering on one side takes place by radiating the net, which is encapsulated or impregnated with resin on one side with UV-light.

The above described method has a great number of advantages. Making the strengthening material self-adhesive as well as the encapsulation or impregnation of the strengthening fibres are carried out in one process. For the manufacturer this means economizing on an additional process in the manufacture of the strengthening material. Because the coating layer and the glue are one product the binding strength of the strengthening fibres of the net with the resin is maximal. For the user the self-adhesive strengthening material according to the invention has the advantage that no extra glue has to be applied. This not only saves the glue but also the operation of applying the glue.

The invention further relates to the strengthening material which can be obtained by means of the method according to the invention. Such a self-adhesive strengthening material comprises for instance a coarse-mesh net consisting of strengthening fibres, which strengthening fibres are at least partially encapsulated or impregnated with an adhesive resin which is made non-adhering on one side of the net, wherein the resin is sensitive to, or can be made sensitive to, UV-light, and making the resin non-adhering on one side takes place by radiating the net, which is encapsulated or impregnated with resin on one side with UV-light. The strengthening material according to the invention can optionally be combined with other strengthening materials, such as threads, non-wovens, membranes, rovings, mats and others. The strengthening material according to the invention is particularly suitable as reinforcement for building materials and in particular for use in road-building, for instance as reinforcement in asphalt.

When the strengthening material according to the invention is fixed to surfaces or walls, it remains lying or hanging in place. This facilitates the processing, whereby it can also be used overhead and against vertical or inclining surfaces. However, as long as no finishing layer of asphalt, cement, plaster, paint, stucco and the like has been applied thereover, the strengthening material can be removed without damage and then fixed once again. This is particularly effective when the surface is dry and dust-free.

Because the strengthening material is non-adhering on one side, it can be supplied for instance as a roll. Because it is non-adhering on one side the strengthening material is moreover not dirtied and does not adhere to machines, material, hands or feet during manufacture or when the finishing layers are applied.

The open net structure ensures that the subsequent finishing layers penetrate well through the strengthening material and anchor it firmly to the base and the subsequent layers. It hereby comes to form part of the whole and can absorb all pressure and tensile forces, shear stresses and the like. The occurrence of cracks as a result of the settling of the ground, for instance in the case of walls, floors, roads etc. is thereby reduced or even prevented. When the strengthening material according to the invention is used in asphalt roads it prevents the rut formation which occurs as a result of road traffic, in particular by trucks during the summer.

In the manufacture of the self-adhesive strengthening material according to the invention a resin is preferably used which can be made partially self-adhesive in one way or other. Particularly recommended is a resin which is sensitive to, or can be made sensitive to, UV light, wherein making the resin non-adhering on one side takes place by radiating the net, which is encapsulated or impregnated with resin, on one side with UV light. Examples of such resins which are UV-sensitive or can be made UV-sensitive are acrylate resins or a mixture of a plurality of acrylate resins with each other or with other types of resin.

The net is for instance a woven fabric or web, and can be manufactured by weaving, knitting, stitching together, tying together or mutually adhering strengthening fibres. The strengthening fibres can have a random mutual angle. Angles between approximately 45° and 90° are recommended. The strengthening fibres forming the net can be threads or rovings, which are manufactured for instance from glass, carbon, aramid, polyester, acryl, polyvinyl alcohol or combinations thereof. The above mentioned materials and net-forming methods are of course only examples which have a particular preference but which can be replaced by the skilled person by equivalents which also fall within the scope of the present invention.

The invention further comprises a method for strengthening building materials, comprising the arrangement of the strengthening material on a base layer and applying thereover one or more finishing layers. The finishing layers can be plaster layers of gypsum or cement, layers of asphalt, concrete, paint, stucco and the like.

The present invention will be further elucidated with reference to the following examples, which are only given by way of illustration and are not intended to limit the invention in any way whatsoever.

### EXAMPLE 1

### Strengthening woven fabric

On a loom a roving of 1 x 600 Tex per centimetre is woven onto a warp consisting of two threads of 272 Tex per centimetre. An open-mesh or coarse-mesh woven fabric hereby results with a mesh size of 1 cm². This woven fabric is subsequently coated with a UV-sensitive self-adhesive acrylate dispersion and after drying irradiated on one side with UV lamps in order to make this side non-adhering.

### EXAMPLE 2

### Self-adhesive strengthening web

On a knitting machine warps of 2400 Tex are knitted to each other every two centimetres with a weft thread of 2400 Tex every centimetre. This open-mesh web is then treated as in example 1.

## Claims

1. Method for manufacturing a self-adhesive strengthening material, comprising the steps of:
a) providing a coarse-mesh net consisting at least partially of strengthening fibres;
b) at least partly encapsulating or impregnating the strengthening fibres of the net with a coating layer of adhesive resin; and
c) making the resin non-adhering on one side of the net, **characterized in that** the resin is sensitive to, or can be made sensitive to, UV light, and making the resin non-adhering on one side takes place by radiating the net, which is encapsulated or impregnated with resin, on one side with UV light.

2. Method as claimed in claim 1, **characterized in that** the resin which is UV-sensitive or can be made UV-sensitive is an acrylate resin or a mixture of a plurality of acrylate resins with each other or with other types of resin.

3. Method as claimed in claims 1 and 2, **characterized in that** providing of the net takes place by weaving, knitting, stitching together, tying together or mutually adhering the strengthening fibres.

4. Method as claimed in claims 1, 2 and 3, **characterized in that** the strengthening fibres forming the net form a mutual angle between 0 and 90°, preferably between 45° and 90°.

5. Method as claimed in any of the claims 1-4, **characterized in that** the strengthening fibres forming the net are threads or rovings, which are manufactured from glass, carbon, aramid, polyester, acryl, polyvinyl alcohol or combinations thereof.

6. Self-adhesive strengthening material comprising a coarse-mesh net consisting of strengthening fibres, which strengthening fibres are at least partially encapsulated or impregnated with an adhesive resin which is non-adhering on one side of the net, **characterized in that** the resin is sensitive to, or can be made sensitive to, UV light, and making the resin non-adhering on one side takes place by radiating the net, which is encapsulated or impregnated with resin, on one side with UV light.

7. Use of a self-adhesive strengthening material as claimed in claim 6, as reinforcement for building materials, in particular for use in road-building.

8. Method for strengthening building materials, comprising of arranging a strengthening material as claimed in claims 6 or 7 on a basis and applying thereover one or more finishing layers.

## Patentansprüche

1. Verfahren zum Herstellen eines selbstklebenden Verstärkungsmaterials, mit den Schritten:
a) Herstellen eines grobmaschigen Netzes, das wenigstens teilweise aus Verstärkungsfasern besteht;
b) wenigstens teilweisem Umkapseln oder Imprägnieren der Verstärkungsfasern des Netzes mit einer Beschichtungsschicht aus klebendem Kunstharz; und
c) Nichtklebendmachen des Kunstharzes an der einen Seite des Netzes,
**dadurch gekennzeichnet, daß** das Kunstharz gegenüber UV-Licht empfindlich ist oder empfindlich gemacht werden kann, und daß das Nichtklebendmachen des Kunstharzes auf der einen Seite stattfindet, indem das Netz, welches mit Kunstharz umgekapselt oder imprägniert ist, an einer Seite mit UV-Licht bestrahlt wird.

2. Verfahren nach Anspruch 1,
**dadurch gekennzeichnet, daß** das Kunstharz, welches UV-empfindlich ist oder UV-empfindlich gemacht werden kann, ein Acrylharz oder ein Gemisch aus einer Anzahl von Acrylharzen miteinander oder mit anderen Arten von Harz ist.

3. Verfahren nach Anspruch 1 und 2,
**dadurch gekennzeichnet, daß** das Herstellen des Netzes durch Weben, Stricken, Zusammennähen, Zusammenbinden oder Zusammenkleben der Verstärkungsfasern erfolgt.

4. Verfahren nach Anspruch 1, 2 und 3,
**dadurch gekennzeichnet, daß** die Verstärkungsfasern, welche das Netz bilden, zueinander einen Winkel zwischen 0 und 90°, vorzugsweise zwischen 45° und 90° bilden.

5. Verfahren nach einem der Ansprüche 1 bis 4,
**dadurch gekennzeichnet, daß** die Verstärkungsfasern, welche das Netz bilden, Fäden oder Vorgarne sind, die aus Glas, Kohlenstoff, Aramid, Polyester, Acryl, Polyvinylalkohol oder Kombinationen derselben hergestellt sind.

6. Selbstklebendes Verstärkungsmaterial mit einem grobmaschigen Netz, bestehend aus Verstärkungsfasern, wobei die Verstärkungsfasern wenigstens teilweise mit einem klebenden Kunstharz umgekapselt oder imprägniert sind, das auf einer Seite des Netzes nichthaftend ist,
**dadurch gekennzeichnet, daß** das Kunstharz gegenüber UV-Licht empfindlich ist oder gemacht werden kann, und das Kunstharz an einer Seite nichthaftend gemacht ist, indem das Netz, welches mit dem Kunstharz umgekapselt oder imprägniert ist, auf einer Seite mit UV-Licht bestrahlt wird.

7. Verwendung eines selbstklebenden Verstärkungsmaterials wie im Anspruch 6 beansprucht, als Verstärkung für Baumaterialien, insbesondere zur Verwendung im Straßenbau.

8. Verfahren zum Verstärken von Baumaterialien, mit Anordnen eines Verstärkungsmaterials nach den Ansprüchen 6 oder 7 auf einer Basis und darauf Aufbringen von einer oder mehreren Fertigstellschichten.

## Revendications

1. Procédé pour fabriquer un matériau de renforcement auto-adhésif, comprenant les étapes de :
a) fournir un réseau à maille grossière constitué au moins partiellement de fibres de renforcement,
b) au moins partiellement encapsuler ou imprégner les fibres de renforcement du réseau avec une couche de revêtement d'une résine adhésive, et
c) rendre la résine non-adhérente d'un côté du réseau, **caractérisé en ce que** la résine est sensible à, ou peut être rendue sensible à, de la lumière UV, et l'étape de rendre non-adhérente d'un côté est assurée en soumettant le réseau, qui est en capsulé ou imprégné avec de la résine, d'un côté à un rayonnement de lumière UV.

2. Procédé selon la revendication 1, **caractérisé en ce que** la résine qui est sensible aux UV ou qui peut être rendue sensible aux UV est une résine acrylate ou un mélange de plusieurs résines acrylates l'une avec l'autre ou avec d'autres types de résine.

3. Procédé selon la revendication 1 ou 2, **caractérisé en ce que** l'étape de fournir le réseau est assurée en tissant, tricotant, cousant ensemble, serrant ensemble ou faisant adhérer ensemble les fibres de renforcement.

4. Procédé selon la revendication 1, 2 ou 3, **caractérisé en ce que** les fibres de renforcement formant le réseau forment un angle mutuel entre 0 et 90°, de préférence entre 45° et 90°.

5. Procédé selon l'une quelconque des revendications 1 à 4, **caractérisé en ce que** les fibres de renforcement formant le réseau sont des fils ou des mèches, qui sont fabriqués à partir de verre, de carbone, d'aramide, de polyester, de composés acryliques, de polyvinyle, d'alcools ou des combinaisons de ceux-ci.

6. Matériau de renforcement auto-adhésif comprenant un réseau à maille grossière constitué de fibres de renfort, lesquelles fibres de renfort sont au moins partiellement encapsulées ou imprégnées d'une résine adhésive qui est non-adhérente d'un côté du réseau, **caractérisé en ce que** la résine est sensible à, ou peut être rendue sensible à, de la lumière UV, et la résine est rendue non-adhérente d'un côté en soumettant le réseau, qui est encapsulé ou imprégné avec de la résine, d'un côté à un rayonnement de lumière UV.

7. Utilisation d'un matériau de renfort auto-adhésif suivant la revendication 6, comme renforcement pour des matériaux de construction, en particulier pour utilisation dans la construction de routes.

8. Procédé pour renforcer des matériaux de construction, comprenant l'agencement d'un matériau de renfort selon la revendication 6 ou 7 sur une base et l'application dessus d'une ou de plusieurs couches de finition.
